

## UNITED STATES PATENT OFFICE

1,986,130

FABRICATION OF ALUMINUM AND ITS  
ALLOYS

Raymond T. Whitzel, Massena, N. Y., assignor to  
Aluminum Company of America, Pittsburgh,  
Pa., a corporation of Pennsylvania

No Drawing. Application March 30, 1932  
Serial No. 602,109

3 Claims. (Cl. 80—60)

This invention relates primarily to the rolling of structural shapes from aluminum base alloys. By the term "structural shapes", I refer, where not otherwise qualified, to wrought products 5 such as are used as materials of construction, widely known in the art by such descriptive terms as angles, I-beams, channels, H-beams, T's, etc. By "structural shapes" I distinguish such shapes as these from members of simple 10 geometric section, such as rectangles, squares, octagons, and the like.

An important object of my invention is to provide a process by which aluminum base alloy structural shapes may be fabricated commercially and a satisfactory product produced consistently, to the end that excessive rejections of faulty material will not burden the operation with high cost. A further important object of 15 the invention is to provide aluminum base alloy structural shapes which are characterized, inter alia, by absence of directional physical properties, so that the shapes will have longitudinal tensile properties substantially the same as those in the transverse direction.

20 Until recently only limited means were available for the production of structural shapes from aluminum base alloys, and the dimensions of the shapes produced were considerably below what were desired in the commercial application of 25 the material. Structural shapes of smaller dimensions were produced by extrusion of the metal but such methods have commercial limitations and the products made were for some uses not wholly satisfactory. With the advent 30 of the use of large ingots and blooms in the rolling of structural shapes of aluminum base alloy, certain unforeseen difficulties developed, among them being a large number of finished shapes which could not be used because of serious 35 defects therein. For instance, in rolling channels from large aluminum alloy blooms, frequent cracking or failure of the piece occurred, thus causing the rejection of a substantial portion of the output of the channel mill.

40 I have discovered that such difficulties were in large part due to insufficient reduction of cross section from the original cast ingot to the bloom, that is, insufficient reduction of cross section prior to the forming of the metal into shapes 45 more complex than the simple geometric forms alluded to. Following this discovery I have developed the method of the present invention, which in its preferred practice consists, briefly, in reducing the section thickness of the original 50 cast ingot by forging or rolling to the extent of 55

at least 80 per cent before attempting to develop, in the worked metal or bloom, the form of the structural shape desired.

In the preferred practice of my invention, the aluminum base alloy ingot should have a sound, 5 clean internal structure, preferably of a uniform and refined grain size, as for example an ingot such as produced by the ingot-casting method described in United States Patent No. 1,777,657, of Stay & Holzhauer, in which method the molten metal in the ingot mold is caused to 10 solidify from the bottom upward in a gradually rising plane, the top portion being the last to solidify. By the method of this patent a cast 15 ingot can be produced which is readily workable and which has an internal structure characterized by substantial uniformity of composition and grain size.

Prior to working the ingot it is given a thermal treatment to develop or impart desirable 20 properties to the metal. In this treatment such factors as temperature, quenching or cooling, aging, etc., will depend (as is well understood in the aluminum alloy arts) upon the specific alloy in question. The temperature of the treatment is usually between about 400 to 550° centigrade. The heated ingot is then delivered to 25 "break-down" or blooming rolls, and at this point the reduction of the cast ingot begins. The complete rolling operation is divided into 30 two stages. In the first the metal is passed back and forth through the blooming rolls, and while maintaining a simple geometric shape the cross section of the original ingot is gradually reduced. In the second stage the rolled metal, as 35 yet in simple geometric cross section, is delivered to the forming rolls, where for the first time the metal is worked to the structural shape desired. Whereas the rolls used in the first or break-down stage have contours designed to produce planar surfaces, the rolls used in the second or forming stage have varying contour, the indentations or projections of one forming roll being so related to the contours of the other 40 that the metal is restricted in all directions except the direction of rolling and must necessarily follow the restricted limitation of the roll design. It is in the first stage of the rolling process and prior to the second or forming stage 45 that in my invention a reduction of at least 80 per cent of the section thickness of the original cast ingot is to be achieved. If the reduction is substantially less than 80 per cent, a large portion of the metal rolled in the second or 50

5

10

15

20

25

30

35

40

45

50

55

forming step will fail, either by cracking, slivering, or the like, thus causing a large number of rejections, with resulting high cost. On the other hand, I have determined that if the reduction is 80 per cent or greater, the failures in subsequent forming to the final shape are in general only such as would be expected in any metal rolling process for producing structural shapes. Moreover, by reducing the section thickness of the original ingot by at least 80 per cent in the first stage, the capacity of the process is considerably increased and aluminum structural members can be fabricated of a size limited only by the size of the ingot and the capacity of the rolling equipment.

Having thus described my invention and the manner in which it may be practiced, I claim:

1. The method of making an aluminum base alloy structural shape comprising casting an ingot, reducing the cross-sectional area of the ingot by mechanical working by at least 80 per cent while maintaining the metal in the form of a simple geometric section devoid of reen-

trant angles, and thereafter developing the final contour of the shape by forming rolls.

2. The method of making an aluminum base alloy structural shape comprising casting an ingot, reducing the cross-sectional area of the ingot at least 80 per cent in a break-down stage by subjecting the metal to the break-down action of rolls having contours designed to produce planar surfaces, and further reducing the cross-section area in a forming stage by 10 subjecting the metal to the action of forming rolls designed to restrict the flow of the metal in all directions except the direction of rolling.

3. The method of making an aluminum base alloy structural shape comprising casting an 15 ingot, reducing the ingot to a bloom, and thereafter developing in the worked metal of the bloom the form of the structural shape desired by subjecting the metal to the action of forming rolls, the reduction in cross-sectional area from 20 the ingot to the bloom being at least 80 per cent.

RAYMOND T. WHITZEL.